

Jan. 16, 1962

J. M. BERRY ET AL

3,017,287

WOOD FINISHING METHOD AND PRODUCT

Filed May 20, 1959

3 Sheets-Sheet 1



FIG-1

INVENTORS  
JOHN M. BERRY  
EVERETTE E. WITT

BY  
*Toulmin & Toulmin*

ATTORNEYS

Jan. 16, 1962

J. M. BERRY ETAL

3,017,287

WOOD FINISHING METHOD AND PRODUCT

Filed May 20, 1959

3 Sheets-Sheet 2



FIG-2

INVENTOR.  
JOHN M. BERRY  
EVERETTE E. WITT  
BY  
*Toulmin & Toulmin*  
ATTORNEYS

Jan. 16, 1962

J. M. BERRY ETAL

3,017,287

WOOD FINISHING METHOD AND PRODUCT

Filed May 20, 1959

3 Sheets-Sheet 3

FIG-3



FIG-4



INVENTOR.  
JOHN M. BERRY  
EVERETTE E. WITT  
BY *Toulmin & Toulmin*  
ATTORNEYS

# United States Patent Office

3,017,287  
Patented Jan. 16, 1962

1

3,017,287

WOODY FINISHING METHOD AND PRODUCT  
John M. Berry, Martinsville, Va., and Everett E. Witt,  
Miamisburg, Ohio, assignors to Midland Chemical Cor-  
poration, Dayton, Ohio, a corporation of Delaware  
Filed May 20, 1959, Ser. No. 814,538  
3 Claims. (Cl. 117—72)

This invention relates to wood finishing systems where-in the wood is provided with a surface adapted for the decoration and preservation of the wood; more particularly the invention relates to wood finishing systems provided to greatly accentuate differences in color between the pore and flake of the wood.

Contrasting shades, and contrasting colorations such as black and white, sometimes termed a sea foam finish, are desired on decorative furniture pieces, and such finishes must also exhibit protective and preservation qualities. Normally aqueous materials are avoided for such purposes, as water stains, for example, tend to raise the grain of the wood, resulting in much labor and expense in overcoming the raised grain effect. Consequently aqueous treating materials have been limited in their application even though the water stains, such as aniline dyes, have long been considered more desirable than the oil and spirit stains.

In the co-pending application of John M. Berry, Serial No. 735,239, filed May 14, 1958, there are described aqueous system wood finishing methods which materially reduce the costs involved while permitting the attainment 30 of the advantages of an aqueous system.

It has now been found that such aqueous methods may be employed in connection with the preparation of wood surfaces having greatly improved contrast between the pore areas and the flake areas of the wood. The system is effective to emphasize naturally occurring differences between the pore and flake as well as to produce contrasting colorations in the pore and flake areas. Further, while flake areas are accentuated the surface is itself smooth and the high labor costs attendant other aqueous systems are eliminated.

Accordingly, a primary object of this invention is to provide an improved economical wood finishing process whereby the naturally occurring differences in the pore and flake areas of the wood are greatly accentuated.

A particular object of the invention is to provide a process which accentuates naturally occurring differences in the pore and flake areas of the wood and which wood may have a clear, pigmented, or contrasting color finish.

In the practice of the method of the copending application referred to hereinbefore the wood treatment involves essentially the application to a smooth wood surface of a fixing agent followed by a filler-sealer coat which provides on the wood a hard, translucent film. Over this film protective lacquer coats or varnish, for example, may be applied.

In the practice of the present invention at least one coloring material is utilized; this coloring material is applied and rag wiped in a glazing operation prior to the application of the filler-sealer which effects the final filling and sealing of the pores of the wood. It may suitably be applied independently of the fixing agent or with the fixing agent.

In instances where two contrasting materials are applied to the wood one is usually applied with the fixing agent and over a first applied coloring material. In any event the wiping operation is effected after the coloring matter is applied and prior to the completion of filling and sealing.

The glazing operation is effective to afford sharp accentuation of the pore areas of the wood and a smooth surface with no grain raising apparent results. To this

2

resultant surface when dry the filler-sealer is applied and cured, and this is suitably followed by the usual finish coats. The product is a hard film on the wood through which the distinctions between the pore and flake areas are apparent in either clear or pigmented finishes.

The invention will be more fully understood by reference to the following detailed description and accompanying drawing wherein:

FIGURE 1 illustrates the steps of the procedure to achieve a black and white (so-called Sea Foam finish);

FIGURE 2 illustrates the steps of the process for attaining a clear finish;

FIGURE 3 illustrates the product;

FIGURE 4 is a diagrammatic, greatly enlarged and fragmentary view of the product illustrating in cross-section a wood surface in accordance with the invention.

The numeral 1 in FIGURES 3 and 4 designates a wood base which has thereon a durable, substantially insoluble, transparent coating designated generally at 2. The coating includes a first film 3 containing a coloring material of whitish coloration and a second film 4 of darker coloration, and a final coating 5 of nitrocellulose lacquer.

## EXAMPLE I

As illustrated in FIGURE 1, to produce a finish having a white background with a dark or black contrasting pore coloration, on mahogany for example, the sanded wood has first applied thereto a light spray of a pigmented vehicle in the general nature of a lacquer toner; this toner provides the desired background color on the wood covering the flake sufficiently to produce a substantially uniform background but without filling the pores to any substantial extent and through which the wood grain is apparent—the wood surface is not therefore completely obscured.

The toner is prepared by diluting one quart of a  $\frac{1}{2}$  second plasticized nitrocellulose solution containing 20 percent nitrocellulose by weight in a lacquer thinner to 1 gallon, and pigmenting the solution with 2 pounds of titanium dioxide by grinding in a pebble mill to secure the dispersion of the dioxide; such toner then may contain:

### Toner "A"

|                                | Parts by weight |
|--------------------------------|-----------------|
| Nitrocellulose                 | 5               |
| Lacquer thinner                | 95 1 gallon.    |
| Plasticizer (dibutylphthalate) | 1               |
| Titanium dioxide               | 2#              |

A light spray of this toner is applied to the wood giving the wood a whitish appearance. The wood is then over dried for about  $\frac{1}{2}$  hour at about 110° F. and then lightly sanded.

A wiping glaze is applied—suitably by spraying—over the wood; this glaze is prepared by first forming an aqueous fixing agent and then pigmenting the fixing agent. The fixing agent contains:

### Fixing agent "A"

|                              |                             |
|------------------------------|-----------------------------|
| Powdered boric acid          | 1.5 lbs.                    |
| Powdered alum                | 1.5 lbs.                    |
| Sucrose (sugar)              | 10 lbs.                     |
| Water                        | 3.5 gallons (29 lbs.).      |
| Wetting agent (Triton X-100) | 6.4 liq. ounces (0.42 lb.). |

The above are mixed together with simple agitation; then 5 liquid ounces of  $H_2SO_4$  (0.63 lb.) are added to yield approximately 5 gallons of the fixing agent "A."

To prepare the glaze:

### Glaze "A"

|                  |        |   |
|------------------|--------|---|
| Fixing agent "A" | gallon | 1 |
| Raw umber        | ounces | 4 |

The fixing agent and umber are mixed with simple agitation.

This glaze is sprayed in a heavy wet coat over the dried white toner. A 3-5 minute air dry period is followed by a wiping of the glaze across the grain of the wood; rag wiping provides a smooth even colored surface with the dark coloring agent-umber in the pores of the wood. This is achieved because the initial light spray of the pigmented toner is insufficient to fill the pores. The dark aqueous coloring agent wipes without disturbing the white undercoat. After wiping, the wood is air dried for approximately 10 minutes and then sprayed with filler sealer.

The filler sealer is also applied by spray and is formed as follows:

*Filler-sealer "A"*

Urea formaldehyde ----- 15#.  
Water ----- 2 gallons (16.6 lbs.).

Mix these components by simple agitation.

Mix:

Sucrose (sugar) ----- 7#.  
Water ----- 0.5 gallon (4.1 lbs.).

and combine the two solutions.

Add:

Glycerine ----- 64 liq. ounces (5.0 lbs).  
Wetting agent (Triton X-100) ----- 6.4 liq. ounces (0.42 lb.).

and mix with simple agitation.

This filler sealer is sprayed over the dried glaze and air-dried for 20-30 minutes, then oven dried for 30-60 minutes at 110° F.-140° F.

The product of the filler-sealer drying is a hard, translucent, smooth film which does not require sanding prior to the application of finish top coats; such finish coats suitably are three coats of a nitrocellulose lacquer; or, alternatively, urea-alkyd varnishes or natural resin varnishes may serve as the finish.

The black coloration in the pores of the wood contrasts sharply with the white background on the wood flake; an important advantage in addition to the appearance of the product is the adhesion of the undercoats to the top coats. This is readily ascertained as by simply puncturing a conventional finish with a knife and stripping the finish peels readily. In contrast the undercoats and top coats of this invention adhere together in a tight bond.

**EXAMPLE II**

To provide a clear finish on walnut, for example, the procedure is similar except that no initial fixing toner is utilized. To the bare sanded wood first apply a glaze made of:

*Wiping glaze "B"*

Fixing agent "A" ----- gal. 0.5  
Raw umber ----- ounces 2

This glaze is sprayed lightly on the wood, is wiped, dried, and the filler sealer "A" and top coats of lacquer are applied, as described in Example I.

The wood finish is transparent, the earth color being left in the wood pores to sharply contrast the pores from the flake area.

**EXAMPLE III**

A glaze for cherry wood contained:

*Cherry glaze*

Fixing agent "A" ----- gal. 0.5  
Burnt umber ----- ounce 1.0  
Burnt sienna ----- do 1.0

The procedure was as in Example II, the cherry glaze being substituted for the walnut.

**EXAMPLE IV**

A glaze for mahogany contained:

*Mahogany glaze*

5 Fixing agent "A" ----- gal. 0.5  
Lemon Iron yellow ----- ounce 0.5  
Burnt umber ----- do 0.5  
Burnt sienna ----- do 0.5

10 The procedure for application is as in Example II, the mahogany glaze being substituted for the walnut.

The glaze in each instance, since it contains the fixing agent, combines the functions of partially filling the pores of the wood without occasioning grain raising to any substantial extent and therefore no sanding is required before applying the fill-seal; the film provided over the wood by the fixing agent is homogeneous, water soluble, continuous and hard; the earth colors of the glaze distribute evenly but are retained substantially only by the pore areas after the wiping. The glaze it itself acidic and reacts with the fill-sealer composition.

The fill-sealer composition wets the dried fixing agent film, provides by virtue of its sugar content some additional filling of the pores and provides a sealing which 25 results in the hard transparent film through which the emphasized differential pore and flake areas are visible.

In the system described the principal function of the sugar is to fill the pores of the wood; in addition the sugar contributes to the viscosity of the liquid necessary for 30 appropriate spraying, and is a further advantage in the formation of a continuous film on the surface of the wood.

The boric acid, sulfuric acid and aluminum sulfate act as acid catalysts for the polymerization of the urea formaldehyde and the filler sealer. Further the boric acid and aluminum sulfate assist in inhibiting grain raising. This grain raising, as already noted, is a common defect in aqueous wood finishing systems.

The wetting agent found to be most desirable is Triton 40 X-100, which is employed in both fixing agent or wiping glaze and the filler sealer, is an alkyl aryl polyether alcohol which is non-ionic. The most suitable wetting agents are those having non-ionic characteristics.

The urea formaldehyde of the filler sealer performs 45 the dual functions of filling and of sealing or insolubilizing. By curing the urea formaldehyde is reacted to form a hard transparent insoluble surface, suitable for the application of lacquer topcoats.

A very suitable urea formaldehyde is that which is 50 sold as a dry partially polymerizable powder having a particle size of about 30 mesh. Other characteristics of such suitable resin include a Stormer viscosity of 20-70 r.p.m. at 21° C. (50 grams of water plus 100 grams of the resin); a gel time at 70° F. of 90-140 minutes (100 grams of the resin and 50 grams 4% ammonium chloride solution).

Glycerin serves as a plasticizer in the filler sealer. It 55 has been found that preferably the weight of glycerin in the filler sealer should be limited to between about 5-10 percent by weight of the filler sealer. Such a plasticizer as the glycerin tends to avoid any crazing of the finished film; with a large excess of the glycerine the rate of cure is reduced.

The coloring agents and pigments employed by the 60 usual commercial trade need not be described in detail.

It will be understood that this invention is susceptible to modification in order to adapt it to different usages and conditions and accordingly, it is desired to comprehend such modifications within this invention as may fall 65 within the scope of the appended claims.

What is claimed is:

1. The process of finishing wood to produce a wood 70 finish surface in which color contrast between the pore and flake areas of the wood is accentuated, comprising the steps of successively treating the wood surface to a

toner, a wiping glaze and an aqueous resin-containing dispersion; said toner being composed of—

|                   |                    |
|-------------------|--------------------|
| Nitrocellulose    | 5 parts by weight  |
| Lacquer thinner   | 95 parts by weight |
| Dibutyl-phthalate | 1 part by weight   |
| Titanium dioxide  | 2 lbs.             |

said wiping glaze being composed of

|                              |                 |
|------------------------------|-----------------|
| Powdered boric acid          | lbs. 1.5        |
| Powdered alum                | lbs. 1.5        |
| Sucrose                      | lbs. 10         |
| Water                        | gal. 3.5        |
| Wetting agent (Triton X-100) | liq. ounces 6.4 |
| Earth color                  | ounces 20       |

and said aqueous resin dispersion being composed of

|                              |                |
|------------------------------|----------------|
| Urea formaldehyde            | lbs. 15        |
| Water                        | gallons 2.5    |
| Glycerin                     | liq. ounces 64 |
| Wetting agent (Triton X-100) | do 6.4         |

2. The process of finishing wood to produce a finish as set forth in claim 1, and wherein said toner is applied to the wood and dried prior to the application of the 25 wiping glaze, and wiping the glaze from the flake area of the wood and into the pore area, applying the resin dispersion thereover, and drying the thus treated wood to produce a hard finish on the wood.

3. The process of finishing wood to produce a wood 30 finish surface in which color contrast between the pore and flake areas of the wood is accentuated, comprising the steps of successively applying to the wood surface to

a wiping glaze and an aqueous resin containing dispersion, said wiping glaze containing—

|                              |                 |
|------------------------------|-----------------|
| Powdered boric acid          | lbs. 1.5        |
| Powdered alum                | lbs. 1.5        |
| Sucrose                      | lbs. 10         |
| Water                        | gal. 3.5        |
| Wetting agent (Triton X-100) | liq. ounces 6.4 |
| Raw umber                    | do 20           |

said aqueous dispersion containing—

|                              |                |
|------------------------------|----------------|
| Urea formaldehyde            | lbs. 15        |
| Water                        | gal. 2.5       |
| Glycerin                     | liq. ounces 64 |
| Wetting agent (Triton X-100) | do 6.4         |

wiping and drying the glaze prior to the application of the dispersion to provide the glaze in the pore area of the wood and to substantially completely remove the glaze from the flake area of the wood, and drying the applied dispersion to a hard insoluble film.

#### References Cited in the file of this patent

##### UNITED STATES PATENTS

|           |                   |               |
|-----------|-------------------|---------------|
| 1,548,528 | Hiltz             | Aug. 4, 1925  |
| 2,015,806 | Menger            | Oct. 1, 1935  |
| 2,565,602 | Fisher et al.     | Aug. 28, 1951 |
| 2,573,105 | Lehman            | Oct. 30, 1951 |
| 2,630,395 | McCullough et al. | Mar. 3, 1953  |
| 2,648,641 | Robison           | Aug. 11, 1953 |

##### OTHER REFERENCES

"Wood Finishing," Vanderwalker, Drake and Co., 1944, pp. 340 and 341.